

1

3,116,278

### WATER-INSOLUBLE AZO-DYESTUFFS

Richard Gross, Frankfurt am Main, and Hasso Hertel and Reinhard Mohr, Offenbach (Main), Germany, assignors to Farbwerke Hoechst Aktiengesellschaft vormals Meister Lucius & Brüning, Frankfurt am Main, Germany, a company of Germany

No Drawing. Filed Apr. 25, 1961, Ser. No. 105,296  
Claims priority, application Germany Apr. 30, 1960

6 Claims. (Cl. 260—146)

The present invention provides new water-insoluble azo-dyestuffs and a process for their manufacture; more particularly it provides new water-insoluble azo-dyestuffs having the general formula



wherein R<sub>1</sub> and R<sub>2</sub> represent hydrogen atoms or alkyl, aryl, aralkyl or cycloalkyl radicals which may be combined to an isocyclic ring, A stands for the radical of an arylamide of an aromatic or heterocyclic o-hydroxycarboxylic acid or of an acylacetic acid, n represents the integer 1 or 2 and the benzene nucleus a may be substituted by groups which do not impart solubility in water.

The invention is based on the observation that new water-insoluble metaliferous azo-dyestuffs are obtained by coupling in substance, on the fiber or on another substratum the diazonium compounds of amines having the general formula



wherein R<sub>1</sub> and R<sub>2</sub> stand for hydrogen atoms or for alkyl, aryl, aralkyl or cycloalkyl radicals which may be combined to an isocyclic ring, the benzene nucleus a may contain substituents which do not impart solubility in water, with arylamides of an aromatic or heterocyclic o-hydroxycarboxylic acid or of an acylacetic acid, the components being selected so that they do not contain groups imparting solubility in water, for example sulfonic acid or carboxylic acid groups, and treating the dyestuffs so obtained with agents yielding metal.

The water-insoluble azo-dyestuffs obtained according to the present invention may be treated in known manner with the agents yielding metal during or after the coupling in substance or on the fiber. When producing the dyestuffs on the fiber the metallization may be carried out by adding agents yielding metal to the developing bath or already to the impregnation bath. The treatment of the dyestuffs with agents yielding metal may be carried out after the coupling in a second bath which is weakly acid, neutral or weakly alkaline and which may contain dispersing agents or detergents, for example a fatty alcohol polyglycol ether, an alkylphenol polyglycol ether, an alkylnaphthol polyglycol ether, a fatty acid polyglycol ester or a fatty acid amide polyglycol ether.

As agents yielding metal, there are preferably used for the process of the present invention compounds yielding copper, cobalt, nickel, manganese, iron, zinc, chromium, aluminum or titanium, which may be used in the form of their mineral or organic salts, such for example as chlorides, bromides, sulfates, nitrates, formates, or as complex compounds of these metals, espe-

2

cially with hydroxy-alkylamines, such for example as diethanolamine, triethanolamine or N-methylethanolamine or with aminocarboxylic acids, such as aminoacetic acid or nitrilotriacetic acid, with aliphatic hydroxycarboxylic acids, such as citric acid, tartaric acid, gluconic acid or glycolic acid, with alkali metal phosphates, such as alkali metal pyrophosphates or alkali metal polyphosphates. When an agent yielding cobalt is used, the addition of compounds of hexavalent chromium or other oxidizing agents, for example alkali metal perborates, alkali metal persulfates or alkali metal percarbonates, has an advantageous effect on the metallization.

On vegetable fibers including fibers of regenerated cellulose there are obtained, according to the dyeing and printing methods known from the ice color industry, metal complex dyestuffs which possess in addition to good general properties of fastness a good fastness to light.

The dyestuffs may be prepared on vegetable fibers in long liquors. Piece goods, chains or ribbons can be dyed continuously or they can be printed according to the methods of base or naphtholate printing.

The new dyestuffs can also be produced on animal fibers, such as wool and silk or on synthetic fibers such, for example as polyamide, acetyl cellulose or polyvinyl alcohol fibers according to the methods used for dyeing these fibers whereby equally interesting dyeings of good fastness properties are obtained.

The dyestuffs can also be prepared in substance and converted into complex metal compounds by treatment with agents yielding metal. The metallization may be carried out in an aqueous solution or in organic solvents such, for example as acetone or dimethylformamide. The metal complex compounds thus obtained are suitable for dyeing animal and synthetic fibers as well as organic plastic masses of high molecular weight.

As coupling components there may be used for the process of the present invention arylamides of aromatic or heterocyclic o-hydroxycarboxylic acids or acylacetic acids, for example arylamides of 2,3-hydroxynaphthoic acid or its derivatives substituted in 6-position, furthermore arylamides of 2-hydroxyanthracene-3-carboxylic acid, 3-hydroxydiphenylene oxide-2-carboxylic acid, 2-hydroxycarbazole-3-carboxylic acid, 5-hydroxy-1,2,1',2'-benzocarbazole-4-carboxylic acid, acetoacetic acid, benzoylacetic acid or terephthaloyl-bis-acetic acid.

As diazo components there may be used compounds having the above general formula which, in the benzene nucleus a may contain substituents which do not impart solubility in water, for example halogen atoms, alkyl, alkoxy, trifluoromethyl, nitro, alkylsulfonic, arylsulfonic and eventually substituted sulfonic acid amide or carboxylic acid amide, acylamino or acyl groups. Such compounds are obtained according to known methods, for example by reacting 3-nitro-1,2-diaminobenzenes with o-diketones, such as glyoxal, diacetyl, benzil, phenanthrenequinone, acenaphthenequinone or 1,2-naphthoquinone and subsequently reducing the nitro group to the amino group. The amines thus obtained represent will crystallizing generally intensely yellow compounds.

The following examples serve to illustrate the invention but they are not intended to limit it thereto:

### EXAMPLE 1

65 Cotton yarn was treated for 45 minutes at 35° C. at a goods-to-liquor ratio of 1:20 in an impregnation bath prepared as described below, then centrifuged, and while wet, developed first for some minutes at 20° C. and then, after being slowly heated to 95° C., for 20 to 30 minutes 70 at 90° C. to 95° C. in a developing bath prepared as described below. The yarn was then rinsed with a solution containing, per liter of water, 3 cc. of hydrochloric

acid of 20 Bé., soaped first for 15 minutes at 60° C. and then for 15 minutes at 95° C. with a solution containing, per liter of water, 1 gram of a reaction product from about 10 mols of ethylene oxide and 1 mol of isododecylphenol, and 3 grams of sodium carbonate, rinsed and dried.

#### Impregnation Bath

1.75 grams of 2-(2',3'-hydroxynaphthoylamino)-naphthalene were dissolved in 3.5 cc. of denatured ethyl alcohol, 0.9 cc. of sodium hydroxide solution of 38° Bé., 2 cc. of warm water and 0.9 cc. of a formaldehyde solution of 30% strength. The solution so obtained was then made up to 1 liter with water at 45° C., 3 grams of a condensation product from fatty acids of high molecular weight and protein degradation products, and 10 cc. of sodium hydroxide solution of 38° Bé.

#### Developing Bath

1.9 grams of 5-amino-2,3,7-trimethyl-quinoxaline in the form of a diazonium compound prepared in the usual manner were dissolved in 1 liter of water containing 2 grams of a reaction product from about 20 mols of ethylene oxide and 1 mol of octadecyl alcohol, 1.5 cc. of acetic acid of 50% strength, 7 grams of sodium acetate and 2.5 grams of copper sulfate.

A garnet dyeing having good properties of fastness was obtained.

By using 2.4 grams of cobalt chloride or 2.8 grams of nickel sulfate instead of 2.5 grams of copper sulfate garnet dyeings equally having good properties of fastness were obtained.

#### EXAMPLE 2

Cotton yarn was treated for 45 minutes at 35° C. at a goods-to-liquor ratio of 1:20 in an impregnation bath prepared as described below, then centrifuged, and while wet, developed for 30 minutes at 20° C. in the developing bath prepared as described below. The yarn was then rinsed with a solution containing, per liter of water, 3 cc. of hydrochloric acid of 20° Bé., soaped for 20 minutes at 95° C. with a solution containing, per liter of water, 1 gram of a reaction product from about 10 mols of ethylene oxide and 1 mol of isododecylphenol, 1 gram of sodium carbonate, 2.5 grams of copper sulfate and 7.5 grams of triethanolamine, rinsed and dried.

#### Impregnation Bath

1.75 grams of 2-(2',3'-hydroxynaphthoylamino)-naphthalene were dissolved in 3.5 cc. of denatured ethyl alcohol, 0.9 cc. of sodium hydroxide solution of 38° Bé., 2 cc. of warm water and 0.9 cc. of a formaldehyde solution of 30% strength. The solution so obtained was then

made up to 1 liter with water at 45° C., 3 grams of a condensation product from fatty acids of high molecular weight and protein degradation products, and 10 cc. of sodium hydroxide solution of 38° Bé.

#### Developing Bath

1.6 grams of 5-amino-7-methyl-quinoxaline in the form of a diazonium compound prepared in the usual manner were dissolved in 1 liter of water containing 2 grams of a reaction product from about 20 mols of ethylene oxide and 1 mol of octadecyl alcohol, 1.5 cc. of acetic acid of 50% strength and 10 grams of sodium acetate.

A violet dyeing having good properties of fastness was obtained.

15 By using in the above example 2.5 grams of cobalt chloride and 11 grams of the sodium salt of nitrilotriacetic acid instead of 2.5 grams of copper sulfate and 7.5 grams of triethanolamine a currant dyeing was obtained and by using 2.8 grams of nickel sulfate and 3 grams of aminoacetic acid a garnet dyeing was obtained.

#### EXAMPLE 3

25 18.7 grams of 5-amino-2,3,7-trimethyl-quinoxaline were dissolved in 500 cc. of ice water and 60 cc. of 5 N-hydrochloric acid. To the deep red solution 20 cc. of a 5 N-sodium nitrite solution were added dropwise at 0° C. to 5° C. After the diazotization the eventually clarified diazo solution was introduced, at 20° C. to 25° C., into a fine suspension prepared from 27.1 grams of 2,3-hydroxynaphthoylaminobenzene of 96.8% strength in a mixture of 1000 cc. of water, 500 cc. of a 2 N-sodium acetate solution and 0.5 grams of a reaction product from about 20 mols of ethylene oxide and 1 mol of oleyl alcohol. After the coupling was terminated the bluish-red dyestuff had precipitated. In order to convert the dyestuff suspension into the complex copper compound a solution containing 25 grams of crystallized copper sulfate in 200 cc. of water and 25 grams of triethanolamine was added and the whole was stirred for some hours at 35° C. to 95° C. until the complex metal compound had completely formed. In the course of this reaction the initially bluish-red suspension became dark red. After the metallization the metal complex compound formed was filtered off with suction at an elevated temperature, washed with hot water and dried. The complex copper compound so obtained was a garnet powder.

30 In the following table further components are listed which can be used in the process of the invention, and the tints produced by forming the metalliferous azo-dye-stuffs from these components on the fibers which tints equally possess good fastness properties.

| Diazo component              | Coupling component                                                  | Tint            |                |                 |
|------------------------------|---------------------------------------------------------------------|-----------------|----------------|-----------------|
|                              |                                                                     | copper complex  | cobalt complex | nickel complex  |
| 5-amino-7-methylquinoxaline. | 2,3-hydroxynaphthoylaminobenzene.                                   | garnet          | currant        | violet.         |
| Do.                          | 1-(2',3'-hydroxynaphthoylamino)-3-nitrobenzene.                     | bluish garnet.  | do.            | reddish violet. |
| Do.                          | 1-(2',3'-hydroxynaphthoylamino)-naphthalene.                        | blue garnet.    | do.            | garnet.         |
| Do.                          | 1-(2',3'-hydroxynaphthoylamino)-4-methoxybenzene.                   | bluish garnet.  | do.            | reddish violet. |
| Do.                          | 1-(2',3'-hydroxynaphthoylamino)-2-methoxy-4-chloro-5-methylbenzene. | do.             | do.            | bluish garnet.  |
| Do.                          | 1-(2',3'-hydroxynaphthoylamino)-2-methoxybenzene.                   | blue garnet.    | do.            | Do.             |
| Do.                          | 1-(2',3'-hydroxynaphthoylamino)-2-methylbenzene.                    | bluish garnet.  | do.            | Do.             |
| Do.                          | 1-(2',3'-hydroxynaphthoylamino)-4-chlorobenzene.                    | do.             | do.            | Do.             |
| Do.                          | 1-(2',3'-hydroxynaphthoylamino)-2-methyl-4-chlorobenzene.           | do.             | do.            | garnet.         |
| Do.                          | 1-(2',3'-hydroxynaphthoylamino)-2-methylmethoxybenzene.             | do.             | do.            | violet.         |
| Do.                          | 1-(2',3'-hydroxynaphthoylamino)-2,4-dimethoxy-5-chlorobenzene.      | reddish violet. | do.            | Do.             |
| Do.                          | 1-(2',3'-hydroxynaphthoylamino)-2,5-dimethoxy-4-chlorobenzene.      | bluish garnet.  | do.            | garnet.         |
| Do.                          | 1-(2',3'-hydroxynaphthoylamino)-2,5-dimethoxybenzene.               | blue garnet.    | do.            | violet.         |

| Diazo component                                  | Coupling component                                                            | Tint            |                  |                     |
|--------------------------------------------------|-------------------------------------------------------------------------------|-----------------|------------------|---------------------|
|                                                  |                                                                               | copper complex  | cobalt complex   | nickel complex      |
| 5-amino-7-methylquinoxaline                      | 1-(2',3'-hydroxynaphthoylamino)-2-ethoxybenzene.                              | bluish garnet.  | curraat.         | garnet.             |
| Do                                               | 2-(2',3'-hydroxynaphthoylamino)-3-methoxy-diphenylene oxide.                  | red violet.     | do.              | Do.                 |
| Do                                               | 1-(6'-bromo-2',3'-hydroxynaphthoylamino)-2-methoxybenzene.                    | blue garnet.    | do.              | violet.             |
| Do                                               | 1-(2',3'-hydroxynaphthoylamino)-2-methyl-5-chlorobenzene.                     | do.             | do.              | bluish garnet.      |
| Do                                               | 1-(2',3'-hydroxyanthracene-3'-carboylamino)-2-methylbenzene.                  | greenish blue   | blue green       | blue garnet.        |
| Do                                               | 1-(2',3'-hydroxynaphthoylamino)-4-ethoxybenzene.                              | bluish garnet.  | currant.         |                     |
| Do                                               | 1-(2',3'-hydroxycarbazole-3'-carboylamino)-4-chlorobenzene.                   | reddish violet. | reddish violet.  |                     |
| 5-amino-2,3-diphenyl-7-methylquinoxaline.        | 2,3-hydroxynaphthoyl-aminobenzene                                             | currant.        | claret.          |                     |
| Do                                               | 1-(2',3'-hydroxy-naphthoylamino)-naphthalene.                                 | do.             | do.              | bluish red.         |
| Do                                               | 2-(2',3'-hydroxy-naphthoylamino)-naphthalene.                                 | do.             | do.              | Do.                 |
| Do                                               | 1-(2',3'-hydroxy-naphthoylamino)-2-methoxy-4-chloro-5-methylbenzene.          | do.             | do.              | Do.                 |
| Do                                               | 1-(2',3'-hydroxy-naphthoylamino)-4-chlorobenzene.                             | do.             | do.              | bluish red.         |
| 5-amino-2,3-naphtho-(1',8')-7-methylquinoxaline. | 1-(2',3'-hydroxy-naphthoylamino)-naphthalene.                                 | do.             | brownish garnet. | bluish covered red. |
| Do                                               | 1-(2',3'-hydroxy-naphthoylamino)-2-methoxy-4-chloro-5-methylbenzene.          | do.             | do.              | Do.                 |
| Do                                               | 1-(2',3'-hydroxy-naphthoylamino)-2-ethoxybenzene.                             | do.             | do.              | covered bluish red. |
| Do                                               | 1-(6'-bromo-2',3'-hydroxynaphthoylamino)-2-methoxybenzene.                    | do.             | do.              | covered claret.     |
| 5-amino-2,3,7-trimethylquinoxaline.              | 2,3-hydroxynaphthoyl-aminobenzene                                             | garnet.         | blue garnet.     | covered red.        |
| Do                                               | 1-(2',3'-hydroxy-naphthoylamino)-3-nitrobenzene.                              | blue garnet.    | do.              | Do.                 |
| Do                                               | 1-(2',3'-hydroxy-naphthoylamino)-4-methoxybenzene.                            | garnet.         | do.              | claret.             |
| Do                                               | 1-(2',3'-hydroxy-naphthoylamino)-2-methoxy-4-chloro-5-methylbenzene.          | blue garnet.    | do.              | covered red.        |
| Do                                               | 1-(2',3'-hydroxy-naphthoylamino)-2-methoxybenzene.                            | garnet.         | garnet.          | Do.                 |
| Do                                               | 1-(2',3'-hydroxy-naphthoylamino)-2-methylbenzene.                             | blue garnet.    | do.              | Do.                 |
| Do                                               | 1-(2',3'-hydroxy-naphthoylamino)-4-chlorobenzene.                             | do.             | blue garnet.     | claret.             |
| Do                                               | 1-(2',3'-hydroxy-naphthoylamino)-2-methyl-4-chloro-benzene.                   | do.             | garnet.          |                     |
| Do                                               | 1-(2',3'-hydroxy-naphthoylamino)-2-methyl-4-methoxy-benzene.                  | blue garnet.    | bluish garnet.   |                     |
| Do                                               | 1-(2',3'-hydroxy-naphthoylamino)-2,4-dimethoxy-5-chloro-benzene.              | do.             | do.              |                     |
| Do                                               | 1-(2',3'-hydroxy-naphthoylamino)-2,5-dimethoxy-4-chloro-benzene.              | do.             | garnet.          | covered red.        |
| Do                                               | 2-(2',3'-hydroxy-naphthoylamino)-3-methoxy-diphenylene oxide.                 | do.             | garnet.          | Do.                 |
| Do                                               | 1-(2',3'-hydroxy-naphthoylamino)-2-methyl-5-chloro-benzene.                   | bluish garnet.  | do.              | Do.                 |
| Do                                               | 1-(2',3'-hydroxy-naphthoylamino)-2-methoxy-5-chloro-benzene.                  | do.             | garnet.          | Do.                 |
| Do                                               | terephthaloyl-bis-(1-acetylamo-2,4-dimethoxy-5-chloro-benzene).               | yellow brown.   | do.              |                     |
| Do                                               | 1-(5'-hydroxy-1',2',1'',2''-benzocarbazole-4'-carboylamino)-4-methoxybenzene. | blue black.     | blue black.      | currant.            |
| Do                                               | 1-(2',3'-hydroxyanthracene-3'-carboylamino)-2-methylbenzene.                  | do.             | currant.         |                     |
| Do                                               | 1-(2',3'-hydroxycarbazole-3'-carboylamino)-4-chlorobenzene.                   | garnet.         | brownish garnet  | brownish garnet     |
| 5-amino-2,3-naphtho-(1',8')-7-methylquinoxaline. | 1-(5'-hydroxy-1',2',1'',2''-benzocarbazole-4'-carboylamino)-4-methoxybenzene. | black.          | do.              |                     |
| Do                                               | 1-(2',3'-hydroxyanthracene-3'-carboylamino)-2-methylbenzene.                  | covered olive.  | do.              |                     |
| Do                                               | 1-(2',3'-hydroxycarbazole-3'-carboylamino)-4-chlorobenzene                    | bluish brown.   | brown.           | reddish brown.      |
| Do                                               | 1-(3'-hydroxylphenylene oxide-2'-carboylamino)-2,5-dimethoxybenzene           | brown.          | reddish brown.   | brown.              |
| Do                                               | terephthaloyl-bis-(1-acetylamo-2,4-dimethoxy-5-chloro-benzene).               | red brown.      | yellow brown.    | yellow brown.       |
| 5-amino-2,3-dimethyl-7-chloroquinoxaline.        | 2,3-hydroxynaphthoyl-aminobenzene                                             | currant.        | flat violet.     |                     |
| Do                                               | 2-(2',3'-hydroxynaphthoylamino)-naphthalene.                                  | do.             | Do.              |                     |
| Do                                               | 1-(2',3'-hydroxynaphthoylamino)-2-methoxybenzene.                             | do.             | garnet.          |                     |
| Do                                               | 1-(2',3'-hydroxynaphthoylamino)-2,4-dimethoxy-5-chlorobenzene.                | do.             | Do.              |                     |
| 5-amino-2,3-dimethyl-7-methoxyquinoxaline.       | 2-(2',3'-hydroxynaphthoylamino)-naphthalene.                                  | garnet.         | garnet.          |                     |

|                    |                                              |       |                   |                     |
|--------------------|----------------------------------------------|-------|-------------------|---------------------|
| Diazo component    | 5-amino-2,3,7-trimethylquinoxaline.          | Tint: | Aluminum complex  | Bluish red.         |
|                    |                                              |       | Chromium complex  | Covered red.        |
|                    |                                              |       | Iron complex      | Covered bluish red. |
| Coupling component | 2-(2',3'-hydroxynaphthoylamino)-naphthalene. | 75    | Manganese complex | Covered red.        |
|                    |                                              |       | Zinc complex      | Covered red.        |
|                    |                                              |       | Titanium complex  | Covered red.        |

We claim:

1. A complex metal compound containing a metal selected from the group consisting of copper, cobalt and nickel, of a water-insoluble azo-dyestuff having the formula



wherein R<sub>1</sub> and R<sub>2</sub> represent individual members selected from the group consisting of a hydrogen atom, methyl group and phenyl group, and R<sub>1</sub> and R<sub>2</sub> represent together a naphthalene radical, X stands for a member selected from the group consisting of a chlorine atom, a methyl group and a methoxy group, Z represents a member of the group consisting of chlorophenyl, nitrophenyl, lower alkylphenyl, lower alkoxyphenyl, naphthyl and the radical of 3-methoxydiphenylene oxide, Y represents the bivalent radical of the group consisting of 2-hydroxynaphthalene-3-carbonylamino-, 6-bromo - 2 - hydroxynaphthalene-3-carbonylamino-, 2-hydroxyanthracene - 3-carbonylamino-, 3-hydroxydiphenylene oxide - 2 - carbonylamino-, 2-hydroxycarbazole - 3 - carbonylamino-, 5-hydroxy-1.2.1'.2'-benzocarbazole - 4 - carbonylamino- and terephthaloyl-bis-acetylaminio-, and n represents one of the integers 1 and 2.

2. The complex nickel compound of the water-insoluble azo-dyestuff having the formula



3. The complex nickel compound of the water-insoluble azo-dyestuff having the formula



4. The complex nickel compound of the water-insoluble azo-dyestuff having the formula



15 5. The complex nickel compound of the water-insoluble azo-dyestuff having the formula



6. The complex nickel compound of the water-insoluble azo-dyestuff having the formula



**References Cited** in the file of this patent

UNITED STATES PATENTS

2,432,419 Heimbach Dec. 9, 1947

#### FOREIGN PATENTS

458,843 Great Britain ----- Dec. 28, 1936